# EUROPEAN PATENT APPLICATION

(11) **EP 2 151 519 A1**
(43) Date of publication of application: **10.02.2010**
(21) Application number: 08465007.6
(22) Date of filing: 30.07.2008
(51) Int. Cl.: D06M 15/00, D06M 15/01

(54) **Method of production of the knitted fabric finished amber appret**

(71) Applicant: Przedsiebiorstwo Wielobranzowe Bowi-Styl, 93-575 Lódz (PL)
(72) Inventor: Sitarz, Wieslawa, 94-043, Lódz (PL)
(74) Representative: Rumpel, Alicja

(57) **Abstract**

The method of manufacturing of the knitted fabric finished with amber finish consisting of the six stages of preparation, bleaching, rinsing, drying, padding bath and final drying. Raw knitted fabric is delivered to the process and prepared for bleaching; next - the knitted fabric is being bleached, preferably in dyeing machine of MCS FIRST type at the temperature close to boiling point of water, preferably at 95°C. During the process of bleaching, a bleaching liquor is applied, where water is used as a carrier of bleaching agents. Bleaching agents are some or all additives falling within the group: hydrogen peroxide solution, caustic soda, stabilizer for hydrogen peroxide solution having a composition and/or properties of SOF FLU preparation, preferably SOF FLU preparation itself, dispersing soap, preferably isol dispersant S40, anti-foam agent having a composition and/or properties of Anchemol P preparation, preferably Anchemol P preparation itself, softening agent and an agent reducing surface tension of the bath and having a composition and/or properties of Softan PE preparation, acetic acid. After completion of bleaching operation, the knitted fabric is being rinsed and dried. Preferably, the drying temperature amounts to about 145°C, whereas the fabric advance speed equals to 10m/min. After drying to the required level of humidity, the knitted fabric passes through the amber padding bath with a squeeze of 60 up to 90%. Preferably, the above is carried out in the apparatus of FULARD type. Besides the dissolved amber, the bath liquor contains also resin having a composition and/or properties of Holiavkiran FEOO preparation and/or bonding hardener having composition and/or properties of Isol thiener PDN. After passing through the padding bath, the knitted fabric reaches the dryer. Preferably, the temperature of drying equals to about 140°C, whereas the fabric advance speed equals to 10m/min.

## Description

The subject-matter of the invention is the method of manufacturing of the knitted fabric with amber finish.

Thanks to its properties both amber and objects made of it are highly valued and used in many fields of life starting from purely decorative function of jewellery made of this fossil resin and ,last but not least, its applications in medicine. In case of medical applications, the most essential properties of amber are its electrostatic properties. It has been observed that amber charges up negatively and that such a way of electrization is a particularly desired method taking into consideration its medicinal properties, e.g. in case of rheumatic diseases.

The medicinal properties of amber in a form of jewellery are ineffective. That is why it is used in a form of ointments, creams, tinctures etc. For therapeutic purposes it is also possible to use woven and knitted fabrics, which contain in their structure particles of amber, charging up negatively the same fabric as well as its close environment.

According to the patent PL 170450, the method of manufacturing of fabric with such properties, consisting in spreading of crushed amber in a form of powder on the surface of fabric or in a form of dispersion in organic solvent has been presented. Concentration of solution to be spread on the surface of material equals to at least 0.005 % by weight of solution, and the solvent in which amber is dissolved boils at the temperature below 200° C. It is also possible to introduce amber onto the surface of material without usage of any solvent. After having been covered with particles of amber, the surface is alternatively pitted or rolled.

A little bit different method of spreading amber on the surface of fabric has been presented in the patent PL170098. The particles of amber with appropriately adjusted weights are added to the reaction mass, from which fibres are received, which are further used in manufacturing of woven or knitted fabrics. In the result of temperature or solvent activity, amber gets into the structure of ready-made product.

The method of manufacturing of knitted fabrics according to the invention enables to eliminate solvents and heating of ready-made product up to the softening temperature of fibres when, at the same time, the particles of amber get into the structure of the product itself.
The method according to the invention consists of six stages.
Stage I - raw knitted fabric is delivered to the process and prepared for bleaching.
Stage II -knitted fabric is being bleached e.g. in dyeing machine of MCS FIRST type. Preferably, every bleaching process is carried out at the temperature close to boiling point of water, preferably at 95°C. During the process of bleaching, a bleaching liquor is applied where water is used as a carrier of bleaching agents. Bleaching agents are some or all additives falling within the group: hydrogen peroxide solution, caustic soda, stabilizer for hydrogen peroxide solution having a composition and/or properties of SOF FLU preparation, preferably SOF FLU preparation itself, dispersing soap, preferably isol dispersant S40, anti-foam agent having a composition and/or properties of Anchemol P preparation, preferably Anchemol P preparation itself, softening agent and an agent reducing surface tension of the bath and having a composition and/or properties of Softan PE preparation, acetic acid. Preferably, when applied in a full range, quantities of bleaching agents are as follows:
   - hydrogen peroxide solution - 10 g/l
   - caustic soda - 2 g/l
   - stabilizer SOF FLU - 0.7 g/l
   - isol dispersant S40 - 0.5 g/l
   - Anchemol P - 1 g/l
   - Softan PE - 3%
   - acetic acid - 1 g/l.
Stage III - After completion of bleaching operation, the knitted fabric is being rinsed. Preferably, rinsing is carried out during at least two cycles. Preferably, an individual cycle of rinsing lasts about 10 minutes.
Stage IV - After it has been stated that residues of bleaching bath have been properly rinsed off, the knitted fabric is being dried. Preferably, the temperature of drying has been adjusted in such a way, that simultaneously with fabric advance speed in relation to the dryer, the optimal drying of the knitted fabric is guaranteed. Preferably, the temperature of drying amounts to about 145°C, whereas the fabric advance speed equals to 10m/min.
Stage V - After drying to the required level of humidity, the knitted fabric passes through the amber padding bath, preferably squeezed from 60% up to 90%. Preferably, the above is carried out in the apparatus of FULARD type. Besides the dissolved amber, the bath liquor contains also resin having a composition and/or properties of Holiavkiran FEOO preparation and/or bonding hardener having a composition and/or properties of Isol thicner PDN preparation. Preferably, in case when both additives are used along with amber, their quantities are as follows:
   - amber - 14 g/l
   - Holiavkiran FEOO - 25 g/l
   - Isol thicner PDN - 5 g/l
   Squeeze from 60 up to 90% means that mass of the knitted fabric after passing through the amber padding bath is larger by 60 up to 90%. Preferably, squeeze is up to 80%.
Stage VI - After passing through the padding bath, the knitted fabric reaches the dryer. Preferably, the temperature of drying has been adjusted in such a way, that simultaneously with fabric advance speed in relation to the dryer, the optimal drying of the knitted fabric is guaranteed. Preferably, the temperature of drying amounts to about 140°C, whereas the fabric advance speed equals to 10m/min.

### Example of making:

The raw knitted fabric delivered for the stage I is prepared for bleaching and then - bleached during the stage II. The knitted fabric is bleached in the dyeing machine of MCS FIRST type, and the process of bleaching is carried out at the temperature close to the boiling point of water i.e. at 95°C. During the process of bleaching the bleaching liquor is applied, where water is used as a carrier of bleaching agents. Bleaching agents are additives falling within the group: hydrogen peroxide solution, caustic soda, stabilizer SOF FLU, isol dispersant S40, Anchemol P, Softan PE, acetic acid and their quantities amount accordingly to:
- hydrogen peroxide solution -10 g/l
- caustic soda - 2 g/l
- stabilizer SOF FLU - 0.7 g/l
- isol dispersant S40 - 0.5 g/l
- Anchemol P - 1 g/l
- Softan PE - 3%
- acetic acid - 1 g/l.
After completion of bleaching operation, the stage III starts during which the knitted fabric is being rinsed. Rinsing is carried out during at least two cycles. An individual cycle of rinsing lasts about 10 minutes. In case of repeated rinsing, each cycle is carried out in a separate bath, which the knitted fabric passes through. After it has been stated that residues of bleaching bath have been properly rinsed off, the knitted fabric is being dried during the stage IV. The temperature equals to about 145°C, whereas the fabric advance speed equals to 10m/min. After drying to the required level of humidity, the stage V of the method according to the invention starts and the knitted fabric passes through the amber padding bath with a squeeze of up to 80%. The above is carried out in the apparatus of FULARD type. Besides the dissolved amber, the bath liquor contains also Holiavkiran FEOO and/or Isol thicner PDN. Their contents are as follows:
- amber - 14 g/l
- Holiavkiran FEOO - 25 g/l
- Isol thicner PDN - 5 g/l
After passing through the padding bath, the stage VI starts during which the knitted fabric reaches the dryer. The temperature of drying equals to about 140°C, whereas the fabric advance speed equals to 10m/min. On completion of drying - ready-made product is formed in bales.

## Claims

1. The method of manufacturing of the knitted fabric finished with amber finish consisting of the six stages of preparation, bleaching, rinsing, drying, padding bath and final drying, **characterized in that** the knitted fabric is bleached in the bleaching liquor, where water used as a carrier of bleaching agents and bleaching agents are some or all additives falling within the group: hydrogen peroxide solution, caustic soda, stabilizer for hydrogen peroxide solution having a composition and/or properties of SOF FLU preparation, dispersing soap, anti-foam agent having a composition and/or properties of Anchemol P preparation, softening agent and an agent reducing surface tension of the bath and having a composition and/or properties of Softan PE preparation, acetic acid; after completion of bleaching operation, the knitted fabric is being rinsed and dried, and then - after drying to the required level of humidity, the knitted fabric passes through the amber padding bath containing dissolved amber and resin having a composition and/or properties of Holiavkiran FEOO preparation and/or bonding hardener having a composition and/or properties of Isol thicner PDN preparation, and after the padding bath - the knitted fabric reaches the dryer.

2. The method according to the claim 1, **characterized in that** SOF FLU preparation is the stabilizer of hydrogen peroxide solution.

3. The method according to the claim 2, **characterized in that** Anchemol P preparation is the anti-foam agent.

4. The method according to the claim 1 or 2 or 3, **characterized in that** Softan PE preparation is the softening agent and an agent reducing surface tension of the bath.

5. The method according to the claim 1 or 2 or 3 or 4, **characterized in that** the process of bleaching is carried out at the temperature close to the boiling point of water.

6. The method according to the claim 1 or 2 or 3 or 4 or 5, **characterized in that** the process of bleaching is carried out at the temperature of 95°C.

7. The method according to the claim 1 or 2 or 3 or 4 or 5 or 6, **characterized in that** in case of application of the full range of bleaching agents, their quantities will be as follows: hydrogen peroxide solution - 10 g/l, caustic soda - 2 g/l, stabilizer SOF FLU - 0.7 g/l, isol dispersant S40 - 0.5 g/l, Anchemol P - 1 g/l, Softan PE - 3%, acetic acid - 1 g/l.

8. The method according to the claim 1 or 2 or 3 or 4 or 5 or 6 or 7, **characterized in that** rinsing is carried out during at least two cycles.

9. The method according to the claim 1 or 2 or 3 or 4 or 5 or 6 or 7 or 8, **characterized in that** an individual cycle lasts about 10 minutes.

10. The method according to the claim 1 or 2 or 3 or 4 or 5 or 6 or 7 or 8 or 9 **characterized in that** the temperature of drying has been adjusted in such a way, that simultaneously with fabric advance speed in relation to the dryer, the optimal drying of the knitted fabric is guaranteed.

11. The method according to the claim 1 or 2 or 3 or 4 or 5 or 6 or 7 or 8 or 9 or 10 **characterized in that** the temperature of drying amounts to about 145°C, whereas the fabric advance speed equals to 10m/min.

12. The method according to the claim 1 or 2 or 3 or 4 or 5 or 6 or 7 or 8 or 10 or 11 **characterized in that** the padding bath is carried out with a squeeze of 60 up to 90%.

13. The method according to the claim 1 or 2 or 3 or 4 or 5 or 6 or 7 or 8 or 10 or 11 or 12 **characterized in that** the padding bath is carried out with a squeeze of up to 80%.

14. The method according to the claim 1 or 2 or 3 or 4 or 5 or 6 or 7 or 8 or 10 or 11 or 12 or 13 **characterized in that** the resin contained in the padding bath is Holiavkiran FEOO preparation.

15. The method according to the claim 1 or 2 or 3 or 4 or 5 or 6 or 7 or 8 or 10 or 11 or 12 or 13 or 14 **characterized in that** the bonding hardener contained in the padding bath is Isol thicner PDN preparation.

16. The method according to the claim 1 or 2 or 3 or 4 or 5 or 6 or 7 or 8 or 10 or 11 or 12 or 13 or 14 or 15 **characterized in that** in case of application of both additives i.e. resin and bonding hardener along with amber, their contents are as follows: amber - 14 g/l, Holiavkiran FEOO - 25 g/l, Isol thicner PDN - 5 g/l.
